

W. H. SOMMER.

**METHOD OF ANNEALING FENCE WIRE.**  
**APPLICATION FILED MAY 7, 1914.**

1,171,673.

Patented Feb. 15, 1916.



# UNITED STATES PATENT OFFICE.

WILLIAM H. SOMMER, OF PEORIA, ILLINOIS.

## METHOD OF ANNEALING FENCE-WIRE.

1,171,673.

Specification of Letters Patent. Patented Feb. 15, 1916.

Application filed May 7, 1914. Serial No. 837,026.

To all whom it may concern.

Be it known that I, WILLIAM H. SOMMER, a citizen of the United States, residing at Peoria, in the county of Peoria and State of Illinois, have invented new and useful Improvements in Methods of Annealing Fence-Wire, of which the following is a specification.

This invention has reference to a new and improved method of annealing fence wire.

Fence wire has been annealed in one of two ways; either by a molten metal process, or by the furnace process. The molten metal process is the more common and more generally used by manufacturers of fence wire.

In drawing wire it becomes stiff and brittle, and to reduce this brittleness and increase flexibility, the wire is annealed by subjecting the same to a temperature, preferably, of about 1,000° to 1,100° Fahr., otherwise the wire will be unfit for fabricating the same into wire fence, barbwire or other purposes, except nails.

The molten metal and furnace processes are inefficient and objectionable, mainly on account of the cost of maintaining a sufficient temperature in the molten metal pans, or furnace, at the point where the wires enter the same. With the molten metal process this is the more objectionable, for the reason, that at times the wire will enter the pans at the freezing point, by this I mean, at or below 32° Fahr., as the room in which the annealing is done usually contains no heat, and if the metal is not kept very hot it will freeze around the wire and cause the wire to break when a splice enters the pan. The furnace process is objectionable for the reason that the temperature is maintained at such a high degree as will cause the wires to become oxidized, should they break and stop within the furnace, creating considerable loss in wire waste, as all that portion of wire stopping within the furnace and becoming oxidized must be scrapped. The molten metal process is less objectionable, in this respect, for the reason, that the wires if broken and stopped in the bath are covered with metal and will not become oxidized, and therefore very little wastes on this account.

One of the objects which I have in view, therefore, is to reduce the cost of annealing wire, by combining with a molten metal

annealing furnace, a pre-heating device through which the wires pass before entering the metal bath, so as to raise the temperature of the wires to as high a point as possible before they enter the bath. This pre-heating device is heated by the waste gases which leave the annealing furnace, but which do not come in contact with the wire, and cost practically nothing, and is therefore a clear gain.

A further object which I have in view, is to provide for heating the pre-heating device with the waste gases from said annealing furnace to a degree which will raise the temperature of the wire previous to its entering the molten metal bath, but which will not be such as to cause oxidizing of the wire in the event of breakage and stopping of the wire in said pre-heating device, thus obviating wire waste in case of breakage and stoppage, as aforesaid.

In the drawings:—Figure 1 is a plan view of an apparatus showing the preferred form by means of which the process may be carried out. Fig. 2 is a longitudinal sectional view, and Fig. 3 is an enlarged cross-section as the same would appear if taken on the line 3—3 of Fig. 1.

1 designates a molten metal annealing furnace containing a number of combustion chambers 2, having connecting gas passages 3. Said furnace is constructed, preferably, with a tunnel 4 leading to a stack 5. 6 and 7 denote pans adapted to contain a suitable molten metal, preferably lead, through which the wires pass. It is preferable to maintain a temperature of about 900° Fahr., in the bath 6, and a temperature of about 1200° Fahr. in the bath 7.

8 designates a pre-heating device connecting with and leading from the annealing furnace 1. This device may be as long as necessity demands and is preferably constructed of fire brick with a gaseous passage 9 therethrough, which communicates with the chambers 2 in the annealing furnace, at one end, see Fig. 2, and with a stack 10, at its outer end. A plurality of spaced supports 11 are arranged in the pre-heating device which support a plurality of wire guiding tubes 12 which open out of the outer and inner walls of said pre-heating device, for the ingress and egress of the wires entering and leaving said pre-heating device.

The wires A are led from suitable reels or supports 13 to and through the tubes 12,

and from said tubes the wires are suitably guided through the molten metal bath in the pans 6 and 7. The waste gases from the chambers 2 in the annealing furnace 1 have 5 two outlets, one through the tunnel 4 and out through the stack 5, and the other through the passage 9 and up and between the supports 11 and tubes 12 and out through the stack 10. The stack 10 is preferably provided with a damper 14, of suitable construction, which regulates the flow of gas through the pre-heating device and thereby determines the temperature therein. By having the two stacks 5 and 10, I obviate 10 the danger of overheating said pre-heating device, which will prevent oxidizing of the wire in the pre-heating device, in the event of breakage and stopping of the wire or wires.

15 In carrying out the invention, the temperature of the waste gases entering and passing through the pre-heating device will produce sufficient heat therein as to raise the temperature of the wires A before they enter the molten metal bath, thus obviating the necessity of maintaining more than just sufficient heat to keep the molten metal in a state or condition to properly and efficiently anneal the wires, and with a 20 minimum cost of fuel, and the fires in the annealing furnace may be replenished at less frequent intervals than heretofore. I can, therefore, anneal the wire at a much lower cost than heretofore, and by raising the temperature of the wires before they 25 enter the metal bath, freezing is entirely obviated. I also obtain all the advantages the use of a molten metal furnace may contain, with less labor and expense, and in

raising the temperature of the wires before they enter the metal bath, do so at little or no expense, and with no danger of oxidizing of the wires in case of breakage and stopping of the wires.

What I claim is:—

1. The herein described method of annealing wire, which consists in passing the wire through an annealing furnace having a combustion chamber and a gaseous passage with a stack leading directly from the chamber 50 and an escape leading from the gaseous passage to provide an escape for waste gases which do not escape through the chamber stack, and previous to such passage, of the wire through the furnace, subjecting such wire to the heat of the waste gases from said furnace in the gaseous passage, without the products of combustion 55 coming into contact with said wire.

2. The herein described method of annealing wire, which consists in passing the wire through a molten metal bath of a furnace having a combustion chamber and a gaseous passage with a stack leading from the chamber and an escape leading from the 65 gaseous passage to provide an escape for waste gases which do not escape through the chamber stack, and previous to the wire entering said bath passing the same through a pre-heater, said pre-heater comprising 70 the gaseous passage being heated by the waste gases from the molten metal bath but without the products of combustion coming into contact with the wire.

WILLIAM H. SOMMER.

Witnesses:

CHAS. W. LA PORTE,  
HAZEL SARSFIELD.